# EUROPEAN PATENT SPECIFICATION

(11) **EP 4 046 515 B1**
(45) Date of publication and mention of the grant of the patent: **09.10.2024**
(21) Application number: 22152740.1
(22) Date of filing: 21.01.2022
(51) Int. Cl.: A41D 19/015, A62B 17/00

(54) **FLAME RETARDANT PROTECTIVE GLOVE**
FLAMMHEMMENDER SCHUTZHANDSCHUH
GANT DE PROTECTION IGNIFUGE

(30) Priority: 01.02.2021 SE 2150111
(43) Date of publication of application: 24.08.2022
(73) Proprietor: Granqvist Sportartiklar AB, 655 91 Karlstad (SE)
(72) Inventor: GRANQVIST, Lars, 655 91 KARLSTAD (SE)
(74) Representative: Bjerkén Hynell KB

(56) References cited:
- DE-A1- 10 111 143
- JP-B2- 6 697 311
- US-A1- 2009 222 980
- US-A1- 2017 280 795
- US-A1- 2019 343 201

## Description

### TECHNICAL FIELD

Flame retardant protective glove, in the form of a finger glove, having an outer shell comprising a back side, a thumb side, an outer side and a palm side, wherein at least the material in the back side, a thumb side and a outer side comprises at least one first multilayer material, comprising an outer layer of a flame retardant material and said palm side comprising a second multilayer material different than said at least one first multilayer material.

### STATE OF THE ART

Flame-retardant protective gloves are a prerequisite for certain professions in order to be able to handle certain occupations that are part of the performance of duties with sufficient security. Examples of such occupational groups are fire fighters, the military, police, ambulance personnel etc. Flameproof gloves are generally known. For example, a protective glove is known from SE 458 254. The protective glove has the shape of a finger glove. The glove consists mainly of leather whose inner surface has been provided with a plastic coating. In addition, the glove is provided with a lining of refractory and heat-insulating material. Such a protective glove becomes relatively awkward due to the plastic-coated leather becoming relatively rigid. In addition, the combination of materials makes it difficult to wash and decontaminate. A similar design is known from DE 10111143 for US 2009/222980.

From US 5,020,161 and WO97/47212, there are known flame-retardant protective gloves that aim at providing similar properties as the glove mentioned above, but without use of leather. A general problem with this known kind of gloves is that the grip in wet conditions may become bad and therefore may jeopardize safety for users. Further, from US 20190343201 there is known a protective garment, e.g. for gloves, that aims at providing protection against noxious gases.

### BRIEF DESCRIPTION OF THE INVENTION

It is an object of the present invention to find a solution to the above-mentioned problem complex, which is achieved by means of a flame retardant protective glove as defined in claim 1.

Thanks to the invention, a flame-retardant protective glove is obtained which in a surprising way at the same time provides good comfort, good protection, good grip ability, good wear resistance and which may securely be washed and decontaminated.

According to a further aspect of the invention:
- the second multilayer material (M2) has a larger elongation at break (ε_{F}) in a length wise direction (F) than the elongation at break (ε_{W}) in a width wise direction (W), which may provide for extra good strength properties of the glove.
- the second multilayer material (M2) has its largest elongation at break (ε_{F}) in a length wise direction (F), whereas the first multilayer material (M1) has its largest elongation at break (ε_{W}) in a width wise direction (W), which may provide for extra good strength properties of the glove.
- second multilayer material (M2) has a tensile strength (σ) of at least 15 daN/5cm in all directions, which may provide for extra good strength properties of the glove.
- The palm side (2) comprises at least one palm part (20) and at least one thumb piece part (61) made of said second multilayer material (M2), which may provide for good ergonomic quality of the glove.
- The at least one first multilayer material (M1, M3) includes a first multilayer material (M1) comprising a basic protective layer (30B) including mainly aramide fibers, suitably Para-aramide fibres, and possibly also other fibres, e.g. polybenzimidazole fibres and a coating comprising silicone, wherein the amount of aramide fibers is larger than the amount of other fibres, e.g. polybenzimidazole fibers, which may provide for an extra good combination of strength and heat resistant of the glove, wherein preferably at least a back side part (30) of the outer shell is made with said first multilayer material (M1) and more preferred also a thumb piece part (61).
- The outer shell includes a third multilayer material (M3) comprising around 50-70 % Polyamide fibers and 30-50% aramide fibers, suitably Para-aramide fibers, preferably the amount of polyamide fibers is larger than the amount of aramide fibers, which may provide a combined outer shell optimizing strength, comfort and heat resistance, wherein preferably at least a plurality of finger side part (70-73) of the outer shell is made with said third multilayer material (M3) and more preferred also at least one hand side part (40, 50).
- an insert (9) is arranged within said outer shell, comprising at least one fire blocker layer (91A, 91B) and at least one aramide fiber containing layer (92), suitably Para-aramide fiber, wherein preferably the insert (9) has a larger amount of fire blocker material (91A, 91B) at the back side (3) than at the palm side (2), more preferred a liquid-tight membrane layer (90), preferable breathable, is arranged in said insert (9).

### BRIEF DESCRIPTION OF FIGURES

In the following, the invention will be described in more detail with reference to the accompanying figures, in which:
Fig. 1 shows a perspective view of a preferred embodiment of a glove according to the invention seen from above,
Fig. 2 shows a perspective view from below of the preferred embodiment of the glove according to the invention,
Fig. 3 shows a cross-sectional view along A-A in Fig. 1,
Fig. 4 shows a cross-sectional view along B-B in Fig. 3,
Fig. 5 shows a preferred embodiment of a back-side part of the preferred embodiment of a glove according to the invention,
Fig. 6 shows a preferred embodiment of a palm-side part of the preferred embodiment of a glove according to the invention,
Fig. 7 shows a preferred embodiment of a first thumb piece part of the preferred embodiment of a glove according to the invention,
Fig. 8 shows a preferred embodiment of a second thumb piece part of the preferred embodiment of a glove according to the invention,
Fig. 9 shows a preferred embodiment of a plurality of parts for the preferred embodiment of a glove according to the invention, one thumb piece part, two side parts and four finger side parts.

### DETAILED DESCRIPTION

Figs. 1 and 2 shows a preferred embodiment of a glove according to the invention from above and below, mainly intended for fire fighters and similar use. The glove is partly made of elastic material, which makes the glove easy to put on and take off and provides good comfort. Through many years of testing of different types of designs and materials, the inventors have arrived at a preferred combination of layers for use in the palm side 2 of an elastic multilayer material, which well meets these complex requirements for fire fighter gloves and similar uses, e.g. meeting the requirements of European standards 420,659 and 388.

In Fig. 1 and Fig. 2 there are shown two perspective views of an exemplary fire figter glove in accordance with the invention. The glove comprises a palm side 2, a backside 3, an outer side 4 and a thumb side 5. The thumb is marked with reference sign 6 and the remaining fingers are given reference number 7. Further, there is shown that the glove also includes a cuff 8.

The glove basically includes three different materials in the outer shell. There is a first material M1 that is used for the backside 3 in the form of a relatively large backside piece 30. There is also a part 60 made in the first material M1 that is used as one of a plurality of pieces for the thumb 6. Further, the first material M1 may also be used for the cuff 8.

The second material M2 is used for the major part 20 of the palm side 2 and also for an inner piece 61 for the thumb 6.

The third material M3 is used in the form of a first side piece 50 on the thumb side 5 of the glove and a second side piece 40 on the outer side 4 of the glove. Furthermore, the third material M3 is used for a plurality of finger side pieces 70, 71, 72, 73. Finally, the third material M3 is used for a third piece 63 of the thumb 6.

There may also be made use of a fourth material 83 for the cuff edge and for the transition zone between the cuff and the glove part. Preferably, made of the same fourth material there is positioned an eyelet device 81 along the palm side of the cuff 8 to assist in putting the glove on.

In Fig. 3 there is shown a cross-sectional schematic view of the glove according to Figs. 1 and 2 along line A-A. It is shown that the glove basically comprises an outer protective shell and an inner protective insert 9. Preferably, the insert 9 is fixated to the outer glove shell by means of seams (not shown) at the fingertip points and also a resilient seam/s 95, preferably Nomex thread, corresponding to a position adjacent the wrist.

In Fig. 4 there is shown a more detailed cross-sectional view along lines B-B in Fig. 3, in order to in more detail explain the different materials used for a glove according to the invention. Firstly, it must be mentioned that the inset 9 may be produced in a large variety of different materials in accordance with the invention, depending on different needs for different uses of a glove according to the invention. In the shown exemplary embodiment the glove is intended for firefighting purposes and provided with preferred combination of materials, without any limitation to such a combination, wherein the combination of materials of the glove 1 may provide protection against harmful biological agents, cuts by hand-held chainsaws, high-pressure jets and bullet wounds or knife stabs.

Starting from the backside 3 there is a first shell material M1 comprising an outer protective layer part 30, se Fig. 5, comprising a basic protective layer 30B and coating 30A. In the shown preferred embodiment the first shell material M1 comprises a basic protective layer 30B including 70-80% aramide fibers, suitably Para-aramide fibres, and 20-30% other strong fibres, e.g. polybenzimidazole fibres, preferably in the form of a half cardigan stitch-knitted fabric. Preferably the aramide fibers are para Aramide fibers. The coating 30A preferably comprises silicone. The weight of the first multilayer material M1 being in the range of 300 - 600 g/m², preferably at least 400 g/m² and a thickness of between 0,8 to 1,8 mm, preferably larger than 1 mm and maximum 1,5 mm. The elongation at break ε is of at least 50% in all directions, preferably at least 70% in all directions. Preferably, the first multilayer material M1 has a larger elongation at break ε_{W} in a width wise direction W than the elongation at break ε_{F} in a length wise direction W, wherein preferably ε_{w} > 1,1 - 2 ε_{F}.

As shown in Figs. 1, 2 and 3 also the cuff piece 80 and a thumb piece part 61 may be made in the same material M1.

As shown in Figs. 1-3 the outer shell of the palm side 2 of the glove comprises two parts 20, 61 made of the second material M2. The large palm part 20, see Fig 5, covers most of the palm of the hand and also includes an inner part for the fingers 7. Preferably also a thumb piece part 61, see Fig 8, is also made of the second material M2, to provide a really good grip.

The second material M2 comprises a multilayer, cohesive material, having an outer coated layer 20B of a flame retardant resilient material comprising Chlorosulfonated Polyethylene and a second, base layer 20A including at least 80% aramide fibers, suitably Para-aramide fibers, preferably at least 90% Para-aramide fibers and more preferred 100% Para-aramide fibers. Preferably the Aramide fibers are para Aramide fibers. The second layer 20A preferably is in the form of an interlock knitted fabric, which provides very good bond for the coated outer layer 20B.

The second material M2 has a surfacic mass of between 400 to 1200 g/m², preferably 500 to 1000 g/m² and a thickness of between 0,5 to 1,5 mm, preferably 0,6 - 1 mm. The elongation at break ε is of at least 20% in all directions, preferably at least 40% in all directions. Preferably, the second multilayer material M2 has a larger elongation at break ε_{F} in a length wise direction F than the elongation at break ε_{W} in a width wise direction W, wherein preferably ε_{F} > 2 ε_{W}, more preferred ε_{F} = 3 - 6 ε_{W}.

The second multilayer material M2 has a tensile strength σ of at least 15 daN/5cm, in all directions, preferably at least 20 daN/5cm, wherein preferably the tensile strength σ_{F} in a length wise direction F is larger than the tensile strength σ_{W} in a width wise direction W, more preferred σ_{F} > 2 σ_{W}, and even more preferred σ_{F} = 3 - 6 ow. Hence, preferably the second multilayer material M2 has its largest elongation at break ε_{F} in a length wise direction F, whereas the first multilayer material M1 has its largest elongation at break ε_{W} in a width wise direction W.

The third material M3 in the outer shell also comprises a multilayer, cohesive material, having an outer layer of a flame retardant material comprising Polyamide fibers and a second layer comprising aramide fibres. Preferably the Aramide fibers are para Aramide fibers. Preferably the third material M3 includes around 50-70 % Polyamide fibers and 30-50% Para-aramide fibers, Preferably the amount of Polyamide fibers is larger than the amount of Para-aramide fibers. The third multilayer material M3 has a surfacic mass of between 300 to 800 g/m², preferably 400 to 600 g/m².

The seams between the parts are preferably made as double seams, and by the use of a sewing thread made from 90-100% spun meta aramid fiber, preferably using a vertically integrated aramid manufacturing system.

As shown in Fig. 4 regarding the insert 9 there is positioned a membrane 90, arranged as an outer layer all around the insert 9. Preferably, it is a copolyamide membrane 90 that is elastic in all directions with high vapor permeability, having a melting temperature above 100 ° C, suitably up to 120° C, and a wash resistance of at least 60° C. Conveniently, the membrane is also completely fogging-free.

Next, the insert 9 at the back side 3 includes two layers 91A, 91B of a heat resistant material, preferably PAN/PES of about 120 to 200 g/m².

Closest to the hand there is a liner 92, preferably including about 50 -70% Aramid and 30-50% glass, of about 250 to 350 g/m².

Moving to the palm side 2 preferably exactly the same layers are being used as for the backside except for using merely one layer 91A of heat resistant material and that the outer shell includes a palm piece 20 that comprises a specific composite layer 20A and a specific coating 20B in accordance with the invention. Hence, the insert 9 preferably has a larger amount of heat resistant material at the back side 3 than at the palm side 2.

Thanks to the invention there is achieved an extremely good grip ability by means of using the novel material M2 in the palm side 2 of the outer shell, e.g. for the pieces 20, 60 at the palm side 2. There has surprisingly been identified that the grip ability when using the material in accordance to the invention is extremely much better than conventional non-leather materials, especially in wet conditions, as presented below.

| GRIP ABILITY | DRY | WET |
|---|---|---|
| Traditional glove using leather in palm side | 5 | 5 |
| Traditional glove using coated textile in palm side | 5 | 2 |
| Glove according to invention | 5 | 5 |

| COMPLIANCY | | DRY | WET |
|---|---|---|---|
| Traditional glove using leather in palm side | | 4 | 5 |
| Traditional glove using coated textile in palm side | | 5 | 5 |
| Glove according to invention | | 5 | 5 |

| WASH ABILITY | DRY |
|---|---|
| Traditional glove using leather in palm side | 3 |
| Traditional glove using coated textile in palm side | 4 |
| Glove according to invention | 5 |

As noted above a glove according to the invention presents a surprising combination of desired properties for a flame retardant glove, for which there has been a long felt need.

The invention is not limited by the above shown but can be varied within the scope of the appended claims. Those skilled in the art will recognize, for example, that the exact design of various components may be varied in many ways. Thus, it is understood, for example, that the glove also retains its basic functionality if having two or more of the fingers integrated to form a common space for two or more fingers, e.g. in the form of a thumb glove.

One variant is, for example, to leave only the index finger and thumb free while the little finger, ring finger and middle finger are combined in a wide finger. Another variant is that only the little finger and ring finger 3 are integrated into one and the same space.

Furthermore, it is understood that materials indicated above with trademarks are only examples of materials with suitable properties and that these can be exchanged for other kinds of materials with the same or similar properties.

## Claims

1. Flame retardant protective glove (1), preferably in the form of a finger glove, having an outer shell comprising a palm side (2), a back side (3), an outer side (4) and a thumb side (5), wherein the material in the back side (3), outer side (4) and a thumb side (5) comprises at least one first multilayer material (M1, M3) comprising an outer layer (30A) of a flame retardant material and said palm side (2) comprises a second cohesive multilayer material (M2) different than said at least one first multilayer material (M1, M3), **characterized in that** said palm side (2) comprises at least one palm part (20) made of said second cohesive multilayer material (M2) having an outer coated layer (20B) of a flame retardant material comprising Chlorosulfonated Polyethylene and a second layer (20A) including at least 80% aramide fibers, suitably para-aramide fibers, wherein said second layer (20A) is in the form of an interlock knitted fabric and said second cohesive multilayer material (M2) has a surfacic mass of between 400 to 1200 g/m², and a thickness of between 0,5 to 1,5 mm, and is resilient having an elongation at break (ε) of at least 20% in all directions.

2. Flame retardant protective glove according to claim 1, **characterized in that** said cohesive second multilayer material (M2) has a larger elongation at break (ε_{F}) in a length wise direction (F) than the elongation at break (ε_{W}) in a width wise direction (W), wherein preferably ε_{F} > 2 ε_{W}, more preferred ε_{F} = 3 - 6 ε_{W}.

3. Flame retardant protective glove according to claim 1 or 2, **characterized in that** said cohesive second multilayer material (M2) has its largest elongation at break (ε_{F)} in a length wise direction (F), whereas the first multilayer material (M1) has its largest elongation at break (ε_{W)} in a width wise direction (W).

4. Flame retardant protective glove according to any of claims 1-3, **characterized in that** said second cohesive multilayer material (M2) has a tensile strength (σ) of at least 15 daN/5cm in all directions, wherein preferably the tensile strength (σ_{F}) in a length wise direction (F) is larger than the tensile strength (αw) in a width wise direction (W), more preferred σ_{F} > 2 σ_{W}, and even more preferred σ_{F} = 3 - 6 σ_{W}.

5. Flame retardant protective glove according to any of claims 1-4, **characterized in that** said palm side (2) comprises at least one palm part (20) and at least one thumb piece part (61) made of said second cohesive multilayer material (M2).

6. Flame retardant protective glove according to any of claims 1-5, **characterized in that** said at least one first multilayer material (M1, M3) includes a first multilayer material (M1) comprising a basic protective layer (30B) including aramide fibers, suitably para-aramide fibres, and other strong fibres, e.g. polybenzimidazole fibres and a coating comprising silicone, wherein the amount of aramide fibers is larger than the amount of other strong fibres, e.g. polybenzimidazole fibers, preferably including 70-80% aramide fibres and 20-30% other strong fibres, e.g. polybenzimidazole fibres, wherein more preferred the weight of said first material (M1) is in the range of 400 - 600 g/m².

7. Flame retardant protective glove according to claim 6, **characterized in that** at least a back side part (30) of the outer shell is made with said first multilayer material (M1) and preferably also a thumb piece part (61), wherein more preferred also a cuff part (80) is made with said first multilayer material (M1).

8. Flame retardant protective glove according to any of claims 6 or 7, **characterized in that** said outer shell includes a third cohesive multilayer material (M3) comprising around 50-70 % Polyamide fibers and 30-50% aramide fibers, suitably para-aramide fibers, preferably the amount of Polyamide fibers is larger than the amount of aramide fibers, more preferred the third cohesive multilayer material (M3) has a surfacic mass of between 300 to 800 g/m², preferably 400 to 600 g/m².

9. Flame retardant protective glove according to claim 6, **characterized in that** at least a plurality of finger side part (70-73) of the outer shell is made with said third cohesive multilayer material (M3) and preferably also at least one hand side part (40, 50), and more preferred also a thumb piece part (62).

10. Flame retardant protective glove according to any proceeding claim, **characterized in that** an insert (9) is arranged within said outer shell, comprising at least one fire blocker layer (91A, 91B) and at least one aramide fiber containing layer (92), suitably para-aramide.

11. Flame retardant protective glove according to claim 10, **characterized in that** said insert (9) has a larger amount of fire blocker material (91A, 91B) at the back side (3) than at the palm side (2).

12. Flame retardant protective glove according to claim 10 or 11, **characterized in that** a liquid-tight membrane layer (90), preferable breathable, is arranged in said insert (9).

13. Flame retardant protective glove according to claim 1, **characterized by** said second layer (20A) including at least 90% aramide fibers and more preferred 100% aramide fibers.

14. Flame retardant protective glove according to claim 1, **characterized by** said second cohesive multilayer material (M2) having a surfacic mass of between 500 to 1000 g/m².

15. Flame retardant protective glove according to claim 1, **characterized by** said second multilayer material (M2) having a thickness of between 0,6 - 1 mm.

## Patentansprüche

1. Schwer entflammbarer Schutzhandschuh (1), vorzugsweise in Form eines Fingerhandschuhs, mit einer Außenhülle, die eine Handflächenseite (2), eine Rückseite (3), eine Außenseite (4) und eine Daumenseite (5) umfasst, wobei das Material auf der Rückseite (3), der Außenseite (4) und einer Daumenseite (5) mindestens ein erstes kohäsives Mehrschichtmaterial (M1, M3) mit einer äußeren Schicht (30A) aus einem flammhemmenden Material, wobei die Handflächenseite (2) ein zweites kohäsives Mehrschichtmaterial (M2) umfasst, das sich von dem mindestens einen ersten kohäsiven Mehrschichtmaterial (M1, M3) unterscheidet, **dadurch gekennzeichnet, dass** die Handflächenseite (2) mindestens ein Handflächenteil (20) aus dem zweiten kohäsiven Mehrschichtmaterial (M2) aufweist, das eine äußere beschichtete Schicht (20B) aus einem flammhemmenden Material umfasst, das chlorsulfoniertes Polyethylen umfasst, und eine zweite Schicht ( 20A) mit mindestens 80 % Aramidfasern, geeignet para-Aramidfasern, wobei die zweite Schicht (20A) in Form eines ineinandergreifenden Gestricks und das zweite kohäsive Mehrschichtmaterial (M2) hat eine Oberflächenmasse zwischen 400 und 1200 g/m2 und eine Dicke zwischen 0,5 und 1,5 mm und ist elastisch mit einer Bruchdehnung (ε) von mindestens 20 % in alle Richtungen.

2. Schwer entflammbarer Schutzhandschuh nach Anspruch 1, **dadurch gekennzeichnet, dass** das kohäsive zweite Mehrschichtmaterial (M2) eine größere Bruchdehnung (εF) in Längsrichtung (F) aufweist als die Bruchdehnung (εW) in breitenweiser Richtung (W), wobei bevorzugt εF > 2 εW, bevorzugter εF = 3 - 6 εW ist.

3. Schwer entflammbarer Schutzhandschuh nach Anspruch 1 oder 2, **dadurch gekennzeichnet, dass** das kohäsive zweite Mehrschichtmaterial (M2) seine größte Bruchdehnung (εF) in Längsrichtung (F) aufweist, während das erste Mehrschichtmaterial (M1) seine größte Bruchdehnung (εW) in Breitenrichtung (W) aufweist.

4. Schwer entflammbarer Schutzhandschuh nach einem der Ansprüche 1 bis 3, **dadurch gekennzeichnet, dass** das zweite bindige Mehrschichtmaterial (M2) eine Zugfestigkeit (σ) von mindestens 15 daN/5cm in allen Richtungen aufweist, wobei vorzugsweise die Zugfestigkeit (σF) in Längsrichtung (F) größer ist als die Zugfestigkeit (σW) in Breitenrichtung (W), bevorzugteres σF > 2 σW und noch bevorzugteres σF = 3 - 6 σW.

5. Schwer entflammbarer Schutzhandschuh nach einem der Ansprüche 1 bis 4, **dadurch gekennzeichnet, dass** die Handflächenseite (2) mindestens ein Handflächenteil (20) und mindestens ein Daumenstückteil (61) aus dem zweiten kohäsiven Mehrschichtmaterial (M2) umfasst.

6. Schwer entflammbarer Schutzhandschuh nach einem der Ansprüche 1 bis 5, **dadurch gekennzeichnet, dass** mindestens ein erstes kohäsives Mehrschichtmaterial (M1, M3) ein erstes kohäsives Mehrschichtmaterial (M1) umfasst, das eine grundlegende Schutzschicht (30B) umfasst, die Aramidfasern, geeignete para-Aramidfasern und andere starke Fasern, z. B. Polybenzimidazolfasern, und eine Beschichtung aus Silikon umfasst, wobei die Menge der Aramidfasern größer ist als die Menge anderer starker Fasern, z. B. Polybenzimidazolfasern, vorzugsweise einschließlich 70-80 % Aramidfasern und 20 bis 30 % andere starke Fasern, z. B. Polybenzimidazolfasern, wobei das Gewicht des ersten kohäsiven Materials (M1) bevorzugter im Bereich von 400 - 600 g/m2 liegt.

7. Schwer entflammbarer Schutzhandschuh nach Anspruch 6, **dadurch gekennzeichnet, dass** mindestens ein hinteres Seitenteil (30) der Außenhülle aus dem ersten bindigen Mehrschichtmaterial (M1) und vorzugsweise auch einem Daumenstückteil (61) hergestellt ist, wobei bevorzugter auch ein Manschettenteil (80) mit dem ersten mehrschichtigen Material (M1) hergestellt ist.

8. Schwer entflammbarer Schutzhandschuh nach einem der Ansprüche 6 oder 7, **dadurch gekennzeichnet, dass** die Außenhülle ein drittes kohäsives Mehrschichtmaterial (M3) umfasst, das etwa 50 bis 70 % Polyamidfasern und 30 bis 50 % Aramidfasern umfasst, geeignet für Para-Aramidfasern, vorzugsweise ist die Menge an Polyamidfasern größer als die Menge an Aramidfasern, bevorzugter das dritte kohäsive Mehrschichtmaterial (M)3 hat eine Oberflächenmasse zwischen 300 und 800 g/m2, vorzugsweise 400 bis 600 g/m2.

9. Schwer entflammbarer Schutzhandschuh nach Anspruch 6, **dadurch gekennzeichnet, dass** mindestens mehrere Fingerseitenteile (70-73) der Außenhülle aus dem dritten kohäsiven Mehrschichtmaterial (M3) und vorzugsweise auch mindestens einem Handseitenteil (40, 50) und bevorzugter auch einem Daumenstückteil (62) hergestellt sind.

10. Flammhemmender Schutzhandschuh nach einem der vorhergehenden Ansprüche, **dadurch gekennzeichnet, dass** innerhalb der Außenhülle ein Einsatz (9) angeordnet ist, der mindestens eine Feuerblockerschicht (91A, 91B) und mindestens eine Aramidfaser enthaltende Schicht (92), geeignet para-Aramid, umfasst.

11. Schwer entflammbarer Schutzhandschuh nach Anspruch 10, **dadurch gekennzeichnet, dass** die Einlage (9) auf der Rückseite (3) eine größere Menge an Feuerblockermaterial (91A, 91B) als auf der Handinnenseite (2) aufweist.

12. Schwer entflammbarer Schutzhandschuh nach Anspruch 10 oder 11, **dadurch gekennzeichnet, dass** in der Einlage (9) eine flüssigkeitsdichte Membranschicht (90), vorzugsweise atmungsaktiv, angeordnet ist.

13. Flammhemmender Schutzhandschuh nach Anspruch 1, **gekennzeichnet durch** die zweite Schicht (20A), die mindestens 90 % Aramidfasern und bevorzugtere 100 % Aramidfasern enthält.

14. Druckfester Schutzhandschuh nach Anspruch 1, **gekennzeichnet durch** das zweite kohäsive Mehrschichtmaterial (M2) mit einer Oberflächenmasse zwischen 500 und 1000 g/m2.

15. Druckfester Schutzhandschuh nach Anspruch 1, **gekennzeichnet durch** das zweite mehrschichtige Material (M2) mit einer Dicke zwischen 0,6 und 1 mm.

## Revendications

1. Gant de protection ignifuge (1), de préférence sous la forme d'un gant à doigts, ayant une coque extérieure comprenant un côté paume (2), un côté arrière (3), un côté extérieur (4) et un côté pouce (5), le matériau de la face arrière (3), de la face extérieure (4) et d'un côté pouce (5) comprenant au moins un premier matériau multicouche cohésif (M1, M3) comprenant une couche extérieure (30A) d'un matériau ignifuge et ledit côté de la paume (2) comprend un second matériau multicouche cohésif (M2) différent dudit au moins un premier matériau multicouche cohésif (M1, M3), **caractérisé en ce que** ledit côté de la paume (2) comprend au moins une partie de la paume (20) constituée dudit second matériau multicouche cohésif (M2) ayant une couche extérieure revêtue (20B) d'un matériau ignifuge comprenant du polyéthylène chlorosulfoné et une seconde couche ( 20A) comprenant au moins 80 % de fibres d'aramide, convenablement des fibres de para-aramide, ladite deuxième couche (20A) se présentant sous la forme d'un tissu tricoté interlock et ledit second matériau multicouche cohésif (M2) a une masse surfacique comprise entre 400 et 1200 g/m2 et une épaisseur comprise entre 0,5 et 1,5 mm, et est élastique avec un allongement à la rupture (ε) d'au moins 20 % dans toutes les directions.

2. Gant de protection ignifuge selon la revendication 1, **caractérisé en ce que** ledit second matériau multicouche cohésif (M2) présente un allongement à la rupture (εF) dans le sens de la longueur (F) que l'allongement à la rupture (εW) dans le sens de la largeur (W), dans lequel de préférence εF > 2 εW, plus préféré εF = 3 - 6 εW.

3. Gant de protection ignifuge selon la revendication 1 ou 2, **caractérisé en ce que** ledit second matériau multicouche cohésif (M2) a son plus grand allongement à la rupture (εF) dans le sens de la longueur (F), tandis que le premier matériau multicouche (M1) a son plus grand allongement à la rupture (εW) dans le sens de la largeur (W).

4. Gant de protection ignifuge selon l'une quelconque des revendications 1 à 3, **caractérisé en ce que** ledit second matériau multicouche cohésif (M2) a une résistance à la traction (σ) d'au moins 15 daN/5cm dans toutes les directions, dans lequel de préférence la résistance à la traction (σF) dans le sens de la longueur (F) est supérieure à la résistance à la traction (σW) dans le sens de la largeur (W), σF > 2 σW préférés, et encore plus préférés σF = 3 - 6 σW.

5. Gant de protection ignifuge selon l'une quelconque des revendications 1 à 4, **caractérisé en ce que** ledit côté de la paume (2) comprend au moins une partie de la paume (20) et au moins une partie du pouce (61) en ce second matériau multicouche cohésif (M2).

6. Gant de protection ignifuge selon l'une quelconque des revendications 1 à 5, **caractérisé en ce que** ledit au moins un premier matériau multicouche cohésif (M1, M3) comprend un premier matériau multicouche cohésif (M1) comprenant une couche protectrice de base (30B) comprenant des fibres d'aramide, de préférence des fibres de para-aramide, et d'autres fibres résistantes, par exemple des fibres de polybenzimidazole et un revêtement comprenant du silicone, la quantité de fibres d'aramide étant supérieure à la quantité d'autres fibres résistantes, par exemple des fibres de polybenzimidazole, comprenant de préférence 70 à 80 % de fibres d'aramide et 20 à 30 % d'autres fibres résistantes, par exemple des fibres de polybenzimidazole, le poids dudit premier matériau cohésif (M1) étant de préférence compris entre 400 et 600 g/m2.

7. Gant de protection ignifuge selon la revendication 6, **caractérisé en ce qu'**au moins une partie arrière (30) de la coque extérieure est réalisée avec ledit premier matériau multicouche cohésif (M1) et de préférence également une partie de pouce (61), de préférence encore une partie de manchette (80) étant réalisée avec ledit premier matériau multicouche (M1).

8. Gant de protection ignifuge selon l'une quelconque des revendications 6 ou 7, **caractérisé en ce que** ladite coque extérieure comprend un troisième matériau multicouche cohésif (M3) comprenant environ 50 à 70 % de fibres de polyamide et 30 à 50 % de fibres d'aramide, de préférence des fibres de para-aramide, de préférence la quantité de fibres de polyamide est supérieure à la quantité de fibres d'aramide, de préférence encore le troisième matériau multicouche cohésif (M3) a une masse surfacique comprise entre 300 et 800 g/m2, de préférence 400 à 600 g/m2.

9. Gant de protection ignifuge selon la revendication 6, **caractérisé en ce qu'**au moins une pluralité de parties côté doigts (70-73) de la coque extérieure sont fabriquées avec ledit troisième matériau multicouche cohésif (M3) et de préférence également au moins une partie côté main (40, 50), et de préférence également une partie pouce (62).

10. Gant de protection ignifuge selon l'une quelconque des revendications précédentes, **caractérisé en ce qu'**un insert (9) est disposé à l'intérieur de ladite coque extérieure, comprenant au moins une couche ignifuge (91A, 91B) et au moins une couche contenant des fibres d'aramide (92), de préférence du para-aramide.

11. Gant de protection ignifuge selon la revendication 10, **caractérisé en ce que** ledit insert (9) présente une plus grande quantité de matériau ignifuge (91A, 91B) sur le côté dos (3) que sur le côté paume (2).

12. Gant de protection ignifuge selon la revendication 10 ou 11, **caractérisé en ce qu'**une couche de membrane étanche aux liquides (90), de préférence respirante, est disposée dans ledit insert (9).

13. Gant de protection ignifuge selon la revendication 1, **caractérisé en ce que** ladite seconde couche (20A) comprend au moins 90 % de fibres d'aramide et de préférence 100 % de fibres d'aramide.

14. Gant de protection ignifuge selon la revendication 1, **caractérisé en ce que** ledit second matériau multicouche cohésif (M2) présente une masse surfacique comprise entre 500 et 1000 g/m2.

15. Gant de protection ignifuge selon la revendication 1, **caractérisé en ce que** ledit second matériau multicouche (M2) présente une épaisseur comprise entre 0,6 et 1 mm.
